

# UNITED STATES PATENT OFFICE.

RENÉ BOHN, OF MANNHEIM, GERMANY, ASSIGNOR TO BADISCHE ANILIN AND SODA FABRIK, OF LUDWIGSHAFEN, GERMANY.

## PROCESS OF DYEING.

SPECIFICATION forming part of Letters Patent No. 681,613, dated August 27, 1901.

Application filed May 27, 1901. Serial No. 62,129. (No specimens.)

*To all whom it may concern:*

Be it known that I, RENÉ BOHN, doctor of philosophy and chemist, a citizen of the Swiss Republic, residing at Mannheim, in the Grand Duchy of Baden, Germany, have invented 5 new and useful Improvements in Processes of Dyeing, of which the following is a specification.

It is known that naphthazarin, a body which 10 has long been used as a dyestuff, yields on reduction a compound which is considered to be tetrahydroxy-naphthalene. (See Zincke and Schmidt, *Annalen der Chemie*, Vol. 286, p. 37.) This body has up to the present not been used 15 or looked upon as a dyestuff, nor has it received any industrial application. I have discovered that it is eminently suited for use as a dyestuff in that it dyes animal fiber directly and combines with metallic mordants, 20 such as alumina or chrome, producing shades which on suitable treatment can be converted into black-lakes of great intensity and fastness. The shade produced on unmordanted wool, for example, is brown, while cotton 25 mordanted with alumina is dyed a yellowish shade, which becomes darker on exposure to air. The dyeings produced on unmordanted material become darker when treated with a suitable oxidizing agent, and if chromates, 30 which are especially suitable, be employed a fast black-lake is formed. The dyestuff on mordanted material is converted into a black metallic lake when treated with bichromate of potash or another suitable oxidizer, which 35 need not contain a chemically - combined metal—for instance, air. The solubility of tetrahydroxy-naphthalene in water is such that the dyeings produced by its aid are of great evenness. At the same time they pos- 40 sess great intensity. The dyeings produced by a given weight of tetrahydroxy-naphthalene and subsequent treatment with chromates are approximately twice as intense as the dyeings produced by the same weight of alizarin-black.

45 In this application for Letters Patent I especially wish to claim the process for producing dyeings by means of tetrahydroxy-naphthalene.

The following examples will serve to further illustrate the nature of my invention and a method of carrying the same into practical effect, but the invention is not confined to the examples. The parts are by weight. 50

*Example 1—Dyeing wool with tetrahydroxy-naphthalene.*—Boil ten (10) kilos of wool in a weak acetic-acid bath for one (1) hour with one hundred and fifty (150) to two hundred (200) grams of tetrahydroxy - naphthalene. Then add one hundred and fifty (150) grams 60 of potassium bichromate and heat for a further three-quarters ( $\frac{3}{4}$ ) of an hour.

*Example 2—Dyeing silk with tetrahydroxy-naphthalene.*—Ten (10) kilos of silk are treated like the wool in Example 1 with the exception that three hundred (300) to four hundred (400) grams of tetrahydroxy-naphthalene are to be employed instead of one hundred and fifty (150) to two hundred (200) grams. 65

*Example 3—Dyeing cotton with tetrahydroxy-naphthalene.*—Boil ten (10) kilograms of cotton mordanted with chrome in an acetic-acid bath for one (1) hour with three hundred (300) grams of tetrahydroxy-naphthalene and then add one hundred and fifty (150) grams 75 of potassium bichromate and boil for a further three-quarters ( $\frac{3}{4}$ ) of an hour.

Now what I claim is—

1. The process of dyeing which consists in treating mordanted textile fiber with tetrahydroxy-naphthalene and subjecting the fiber thus treated to the action of oxidizing agents, substantially as described. 80

2. The process of dyeing which consists in treating textile fiber with tetrahydroxy-naphthalene and subjecting the fiber thus treated to the action of oxidizing agents, substantially as described. 85

In testimony whereof I have hereunto set my hand in the presence of two subscribing witnesses. 90

RENÉ BOHN.

Witnesses:

JOHN L. HEINKE,  
PERCY J. JONES.